

## UNITED STATES PATENT OFFICE.

SETH F. WATSON, OF RICHMOND, INDIANA, ASSIGNOR OF ONE-HALF HIS  
RIGHT TO JAMES H. McMURTRY.

## IMPROVEMENT IN FIRE-KINDLERS.

Specification forming part of Letters Patent No. 124,705, dated March 19, 1872.

## SPECIFICATION.

Know all men by these presents that I, SETH F. WATSON, of the city of Richmond, State of Indiana, have invented a certain Compound called The American Fire-Kindling, to be used for starting wood, coal, and other fires in place of shavings and other kindlings.

My invention consists in compounding together tallow, rosin, saw-dust, coal-dust, dissolved glue, and petroleum, and preparing the composition for use in the manner hereinafter specified.

To prepare about one hundred pounds of my American fire-kindling, I melt about eight and one-half pounds of tallow in a suitable vessel, and, when hot, add to it about forty-three pounds of rosin and melt the same. I then add about twenty-three pounds of dry saw-dust, pine being preferable; but other kinds may be used. I next add about sixteen pounds of coal-dust or refuse fine coal from a good quality of coal; meanwhile, all the articles are thoroughly mixed together. I next add about two and one-half pounds of glue previously dissolved in sufficient water to make it about the consistency of milk. I next add about seven

pounds of crude petroleum, and stir so as to mix all the ingredients thoroughly. I then let it cool until it is as cold as can be worked conveniently. I next press it out in broad sheets in a press, previously placing a layer of dry saw-dust on the bottom of the press of sufficient thickness to prevent the materials from sticking to the press. I then place on the press sufficient of the material to make a broad sheet about one inch thick. I next sprinkle sufficient dry saw-dust on it to keep it from sticking to the press, and press it to the desired thickness and density. I then remove from the press and cut into pieces about one and one-half inches square, one piece of which is sufficient to kindle any ordinary wood or coal fire.

I claim as my invention—

The composition herein specified, consisting of the ingredients named, and prepared in the manner described.

SETH F. WATSON.

## Witnesses:

M. C. THOMPSON,  
J. M. SUFFRINS.